



US006273178B1

(12) **United States Patent**  
Osada et al.

(10) **Patent No.:** US 6,273,178 B1  
(45) **Date of Patent:** Aug. 14, 2001

(54) **TWIN ROLL CONTINUOUS CASTING INSTALLATION**

5,385,201 \* 1/1995 Praeg ..... 164/480

(75) Inventors: **Shiro Osada**, Yokohama; **Osamu Takeuchi**, Mataka; **Atsushi Hirata**, Hiratsuka, all of (JP)

**FOREIGN PATENT DOCUMENTS**

3-291135 \* 12/1991 (JP) ..... 164/428  
5-318047 \* 12/1993 (JP) ..... 164/428

(73) Assignees: **Ishikawajima-Harima Heavy Industries Company Limited**, Tokyo (JP); **BHP Steel (JLA) Pty. Ltd.**, Melbourne (AU)

\* cited by examiner

(\*) Notice: Subject to any disclaimer, the term of this patent is extended or adjusted under 35 U.S.C. 154(b) by 0 days.

(21) Appl. No.: **09/553,318**

(22) Filed: **Apr. 20, 2000**

*Primary Examiner*—Nam Nguyen

*Assistant Examiner*—I-H. Lin

(74) Attorney, Agent, or Firm—Miles & Stockbridge P.C.; John C. Kerins

(57) **ABSTRACT**

The invention addresses the problem of edge bulging and breakout of as cast strip due to a decrease of perfect solid phase shell thickness of the strip caused by heat recuperation of the unsolidified portion of the strip, by providing a chamber 19 which encloses the travel path of a strip 8 delivered from a pair of chilled rolls 1a and 1b, a pair of chilled blocks 29a arranged in the chamber to be positioned near a nip between the chilled rolls 1a and 1b, with each chilled block 29a being shaped for loose fitting over an edge of a strip 8 and being capable of injecting cooling gas toward the edge of the strip 8. When the strip 8 is to be continuously cast, the interior of the chamber 19 provides an inert gas atmosphere, in which the cooling gas injected by the cooling blocks 29a injection-cools the edges of the strip 8 delivered from the chilled rolls 1a and 1b at a position near the nip between the chilled rolls 1a and 1b.

(63) Continuation of application No. 09/100,348, filed on Jun. 19, 1998, now Pat. No. 6,079,479.

**Related U.S. Application Data**

(30) **Foreign Application Priority Data**

Jun. 23, 1997 (AU) ..... PO7496

(51) **Int. Cl. 7** ..... B22D 11/06; B22D 11/24

(52) **U.S. Cl.** ..... 164/480; 164/428; 164/414; 164/444

(58) **Field of Search** ..... 164/480, 428, 164/444, 414

(56) **References Cited**

**U.S. PATENT DOCUMENTS**

4,658,882 \* 4/1987 Oba et al. ..... 164/414

**6 Claims, 7 Drawing Sheets**















**PRIOR ART**FIG. 8.FIG. 9.**PRIOR ART**

## TWIN ROLL CONTINUOUS CASTING INSTALLATION

### CROSS-REFERENCE TO RELATED APPLICATION

This application is a con of Ser. No. 09/100,348, filed on Jun. 19, 1998 and now issued as U.S. Pat. No. 6,079,479.

### FIELD OF THE INVENTION

The present invention relates to a twin roll continuous casting installation wherein molten metal is quenched for solidification and directly molded into a metal sheet.

### Prior Art

It is known in the art of continuous casting that quenching of poured molten metal for solidification into a strip will greatly improve characteristics of the material owing to formation of stable phase in the strip, drastic reduction of microsegregation and micronization of the structure and the like.

For casting such strip, there have been proposed installations in which molten metal is poured into a nip between a pair of chilled roll to be quenched into a strip.

Problems during the pouring and quenching of molten metal are deteriorated cleanliness of the molten metal due to oxygen in surrounding atmosphere as well as formation of oxidized scale on the strip.

A proposal for overcoming the problems is disclosed in JP-B-3-33053.

FIG. 7 shows a twin roll continuous caster as disclosed in this Japanese patent publication. It comprises an upstream chamber 2 constituting a main-body vessel and a downstream chamber 12 disposed just below the chamber 2 and constituting a strip-delivering vessel. Prior to continuous casting of strip (strip 8), interiors of the chambers 2 and 12 are substituted into inert gas atmospheres.

Arranged in the upstream chamber 2 in the order named from above are a tundish 5, a pair of chilled rolls 1a and 1b and a pair of upper cooling gas sprays 10a and 10b. Molten metal supplied from a ladle 7 outside and above the upstream chamber 2 to the tundish 5 is poured into the nip between the chilled rolls 1a and 1b which are rotated, so that the molten metal is cooled by the rolls 1a and 1b into solidified strip 8 which is continuously delivered downward.

The strip 8 delivered by the chilled rolls 1a and 1b is cooled at its opposite surfaces by inert gas injected by the upper cooling gas sprays 10a and 10b and passed to the downstream chamber 12.

Arranged in the downstream chamber 12 in the order named from above are a pair of lower cooling gas sprays 15a and 15b and a pair of pinch rolls 11a and 11b. The strip 8 delivered from the upstream chamber 2 is cooled at its opposite surfaces by inert gas injected from the lower cooling gas sprays 15a and 15b and is passed outside of the downstream chamber 12.

Thus, the twin roll continuous casting installation shown in FIG. 7 suppresses deteriorated cleanliness of the molten metal and prevents oxidization of the strip surfaces in such a manner that the interiors of the upstream and downstream chambers 2 and 12 are substituted into inert gas atmospheres and the inert gas is injected to the opposite surfaces of the strip by the gas sprays in the chambers 2 and 12.

Meanwhile, a recent problem on strip in continuous casting is occurrence of bulging on the strip at its widthwise

edges (edge bulging), break on the strip at the edges (edge break) and strip fracture (breakout) due to a phenomenon that insufficient cooling on the strip at its widthwise edges may result in the unsolidified surface of the strip just after the casting being melted again because of heat recuperation. A proposal to overcome the problem is disclosed in JP-A-5-277654.

FIGS. 8 and 9 show a twin roll continuous caster disclosed in this publication and having a pair of dog bone type chilled rolls 17a and 17b rotatably arranged below the chilled rolls 1a and 1b. The chilled rolls 17a and 17b have, at their opposite ends, enlarged roll portions which contact widthwise opposite edges on opposite surfaces of the strip 8 from the chilled rolls 1a and 1b, so that the widthwise edges of the strip 8 just after the casting is quenched to prevent edge break of the strip 8.

However, in the twin roll continuous caster as disclosed in JP-B-3-33053 (see FIG. 7), sealing of the upstream and downstream chambers 2 and 12 for maintaining the inert gas atmospheres in casting of the strip 8 will elevate temperatures in the chambers 2 and 12, so that the strip 8 must be cooled by the upper cooling gas sprays 10a and 10b below the chilled rolls 1a and 1b. Since the inert gas from the sprays 10a and 10b is injected over the whole surfaces of the strip 8, cooling effect may be low at the widthwise opposite edges of the strip 8, disadvantageously resulting in occurrence of edge bulging.

On the other hand, in the twin roll continuous caster as disclosed in JP-A-5-277654 (see FIGS. 8 and 9), assumption in actual operation may be made such that the chilled rolls 1a and 1b have outer diameter of 400–600 mm and the enlarged portions of the dog bone type chilled rolls 17a and 17b have outer diameter of 200 mm. Then, the distance of the dog bone type chilled rolls 17a and 17b from the chilled rolls 1a and 1b may be 300–400 mm, which may cause insufficient cooling effect on the widthwise opposite edges of the strip 8 just below the nip between the chilled rolls 1a and 1b, disadvantageously resulting in occurrence of edge bulging and breakout on the strip 8.

Further, the inventors experimentally investigated a relationship of perfect solid phase shell thickness near the edge of the strip 8 to distance of the chilled rolls 1a and 1b from the nip between the chilled rolls 1a and 1b in the manufacturing conditions that, as shown in FIG. 6, atmosphere temperature in the chamber is 1200°C., strip thickness is 2 mm and manufacturing speed is 60 m/min. As a result, it was found out that, in the condition ① in the Figure where no cooling is effected, the perfect solid phase shell thickness of the edge of the strip 8 tends to decrease to zero due to heat recuperation of unsolidified portion in the strip 8 so that edge bulging, edge break and/or breakout of the strip 8 is likely to occur on such portion.

The present invention was made in view of the above and has an object to provide a twin roll continuous casting installation which can alleviate decrease of the perfect solid phase shell thickness near the edge of the strip caused by heat recuperation of the unsolidified portion.

### SUMMARY OF THE INVENTION

According to the invention there is provided a twin roll continuous casting installation comprising pinch rolls for clamping a strip continuously cast by a pair of chilled rolls, a chamber for enclosing travel path of the strip from the chilled rolls to the pinch rolls, said chamber having seal members airtightly in contact with outer peripheries of the chilled rolls and pinch rolls, and a pair of chilled blocks for

injecting cooling medium to edges of the strip delivered from the chilled rolls, said blocks being shaped for loose fitting over the edges of the strip, one of the blocks being arranged just below one ends of the chilled rolls, the other block being arranged just below the other ends of the chilled rolls.

It is preferred that each of the chilled blocks has cooling medium passages therein to cool the chill blocks.

Preferably each of the pair of chilled blocks is adapted to be moved between a position where the chilled block is loosely fitted over the edge of the strip just below the chilled rolls and a position where the chilled block is not affected by splashing of metal dropping from the nip between the chilled rolls at the beginning of strip casting.

It is preferred that cooling gas is injected from the pair of blocks toward the edges of the strip positioned near the nip between the chilled rolls, thereby preventing decrease of perfect solid phase shell thickness of the strip due to heat recuperation of unsolidified portion to suppress edge bulging and breaking of the strip.

Preferably cooling medium is passed through cooling medium passages of the respective chilled blocks to enable radiation-cooling of the edges of the strip positioned near the nip between the chilled rolls by the blocks, thereby preventing decrease of perfect solid phase shell thickness of the strip due to heat recuperation of the unsolidified portion to more effectively suppress edge bulging and edge breaking of the strip.

It is preferred that each of the pair of chilled blocks is displaced to a position where the chilled block is not affected by splashing of molten metal dropping from the nip between the chilled rolls, thereby preventing the chilled block from being damaged.

#### BRIEF DESCRIPTION OF THE DRAWINGS

In order that the invention may be more fully explained one particular embodiment will be described in detail with reference to the accompanying drawings in which:

FIG. 1 is a schematic view, looking from one end side of the chilled rolls, of an embodiment of a twin roll continuous casting installation according to the invention;

FIG. 2 is a view looking in the direction of the arrows II-II in FIG. 1;

FIG. 3 is a view looking in the direction of the arrows III-III in FIG. 1;

FIG. 4 is a detailed, cross sectional view of the chilled block shown in FIGS. 1 to 3;

FIG. 5 is a view looking in the direction of the arrows V-V in FIG. 4;

FIG. 6 is a graph showing a relationship of perfect solid phase shell thickness at the edge of a strip to distance from nip between chilled rolls in the twin roll continuous casting installation shown in FIG. 1;

FIG. 7 is a schematic view of a twin roll continuous caster disclosed in JP-A-3-33053;

FIG. 8 is a schematic view of a twin roll type thin sheet continuous caster disclosed in JP-A-5-5277654; and

FIG. 9 is view looking in the direction of arrows IX-IX in FIG. 8.

#### DETAILED DESCRIPTION OF THE PREFERRED EMBODIMENT

A preferred embodiment of the present invention will be described in conjunction with the attached drawings.

FIGS. 1 to 5 show an embodiment of a twin roll continuous casting installation of the invention where the same components as in FIGS. 7 to 9 are referred to by the same reference numerals.

Reference numerals 16 and 16b represents a pair of side weirs. One side weir 16a is positioned to have surface contact with one end surfaces of chilled rolls 1a and 1b. The other side weir 16b is positioned to have surface contact with the other end surfaces of the chilled rolls 1a and 1b. A molten metal pool 6 is formed in a space defined by the chilled rolls 1a and 1b and the side weirs 16a and 16b.

Reference numerals 18a and 18b represent a pair of pinch rolls which are positioned horizontally on one side below the chilled roll 1a so that a strip 8 from the chilled rolls 1a and 1b may be clamped from above and below.

Reference numeral 19 represents a chamber which is formed to enclose travel path of the strip 8 from the chilled rolls 1a and 1b to the pinch rolls 18a and 18b.

This chamber 19 is formed, at its portions just below the side weirs 16a and 16b, with pockets 19a and 19b for standby of below-mentioned chilled blocks 29a and 29b, respectively.

Arranged in positions on the chamber 19 are an inert gas supply port 20 for supplying inert gas as non-oxidizing gas to the chamber 19 as well as a discharge port 21.

Reference numerals 22a and 22b represent seal members which are mounted at an end of the chamber 19 facing the chilled rolls 1a and 1b so that the seal members 22a and 22b airtightly contact outer peripheries of the chilled rolls 1a and 1b.

Reference numerals 23a and 23b represent seal members which are mounted to an end of the chamber 19 facing the pinch rolls 18a and 18b so that the seal members 23a and 23b airtightly contact outer peripheries of the pinch rolls 18a and 18b.

As these seal members 22a, 22b, 23a and 23b, labyrinth seal or wire seal comprising a number of metal stands may be used.

Reference numerals 24a and 24b represent a pair of cylinders for withdrawal. The cylinders 24a, 24b comprises a cylinder body 25a, 25b which is mounted on an outer side of the pocket 19a, 19b of the chamber 19 via a bracket 26a, 26b such that it is positioned in parallel with rotary axes xa and xb of the chilled rolls 1a and 1b.

The cylinders 24a, and 24b has a piston rod 27a, 27b which extends via a seal member 28a, 28b through the pocket 19a, 19b of the chamber 19. The piston rod 27a, 27b has a tip which is adapted to be moved toward or away from the edge 8a, 8b of the strip 8 positioned near the nip between the chilled rolls 1a and 1b when fluid pressure is applied to a head- or rod-side fluid chamber of the cylinder body 25a, 25b.

The cylinders 24a and 24b may be designed such that fluid pressure is simultaneously applied to their head- or rod-side fluid chambers; alternatively, the cylinders 24a and 24b may be designed to be applied with fluid pressure independently from each other.

Reference numerals 29a and 29b denote a pair of chilled blocks each of which has a notch 30a, 30b extending from a distal end toward a proximal end of the block so that it may be loosely fitted over the edge 8a, 8b of the strip 8 (see FIG. 4).

With the chilled block 29a, 29b being loosely fitted over the edge 8a, 8b of the strip 8, a cooling gas passage 31a, 31b extends through the chilled block 29a, 29b from a proximal end surface thereof to the notch 30a, 30b; and cooling medium passages 32a, 32b extend through the block 29a, 29b from the proximal end surface thereof via vicinity of the distal end thereof back to the proximal end thereof.

The chilled block 29a, 29b is arranged in the pocket 19a, 19b of the chamber 19.

The piston rod 27a, 27b of the withdrawal cylinder 24a, 24b is fixed at its tip to the proximal end face of the chilled block 29a, 29b. Displacement of said piston rod 27a, 27b will cause the chilled block 29a, 29b to be moved between a position where the chilled block is loosely fitted over the edge 8a, 8b of the strip 8 delivered from the chilled rolls 1a and 1b and a position where the chilled block is not affected by splashing of molten metal dropping from the nip between the chilled rolls 1a and 1b at beginning of casting of the strip 8.

Arranged near the chilled block 29a, 29b is a monitor camera (not shown) for ascertaining whether splashing of molten metal at the beginning of the strip casting has ceased or not so that an operator may confirm internal condition of the chamber 19.

The above-mentioned chilled blocks 29a and 29b may be produced by sequentially performing machining operations such as cutting, drilling and partial hole-filling of metal material; alternatively, they may be produced by precision integrated casting using lost wax technique.

A nitrogen gas (inert gas) storage vessel (not shown) which serves as cooling gas supply source is connected to an proximal end (an end on the proximal end surface of the chilled block 29a, 29b) of the cooling gas passage 31a, 31b, nitrogen gas being injected through the chilled block 29a, 29b.

A cooling water vessel (not shown) which serves as cooling medium supply source is connected through a cooling medium supply pipe (not shown), which airtightly passes through the chamber 19 and is flexible, and through a water supply pump (not shown) to one end of the cooling medium passage 32a, 32b. The other end of the passage 32a, 32b is connected through a cooling medium recovery pipe (not shown), which airtightly passes through the chamber 19 and is flexible, and through a heat exchanger (not shown) to the above-mentioned cooling water vessel. Thus, cooling water will continuously flow through the cooling medium passage 32a, 32b.

Flowing of the cooling water through the cooling medium passage 32a, 32b is not limited to the above-mentioned circulating technique. Alternatively, the cooling water may merely pass through the passage without circulating.

Reference numeral 33 represents a sledding table in the form of curved plate when viewed axially of the chilled rolls 1a and 1b.

The sledding table 32 is arranged in the chamber 19 below the chilled rolls 1a and 1b and the chilled blocks 29a and 29b so that the table 32 may be swung between a guide position (the condition shown by two-dot chain line in FIG. 1) where the table 32 guides substantially horizontally the strip 8 from the chilled rolls 1a and 1b toward the above-mentioned pinch rolls 18a and 18b and a standby position (the condition shown by solid line in FIG. 1) hanging downward from the guide position.

Next, mode of operation of the twin roll continuous casting installation shown in FIGS. 1 to 5 will be described.

When the strip 8 is to be continuously cast by the chilled rolls 1a and 1b, prior to the casting of the strip 8, nitrogen gas is charged into the chamber 19 through the supply port

20 and discharge through the discharge port 21 is made to some extent to maintain the interior pressure, thereby turning the interior of the chamber 19 to a non-oxidizing gas atmosphere (inert gas atmosphere).

5 Each of the chilled blocks 29a and 29b is withdrawn by the cylinder 24a, 24b to a standby position where the chilled block is not affected by splashing of the molten metal dropping from the nip between the chilled rolls 1a and 1b at the beginning of casting of the strip 8, and the cooling water is preliminarily passed continuously through the cooling medium passage 32a, 32b of the chilled block 29a, 29b; and the sledding table 33 is swung to the above-mentioned guide position.

Upon completion of the preparations as described above, the molten metal is supplied to a space defined by the chilled rolls 1a and 1b and the side weirs 16a and 16b to form the molten metal pool 6. Then, the chilled rolls 1a and 1b positioned at right and left in FIG. 1 are rotated clockwise and counterclockwise, respectively, at the same time.

When splashing of the molten metal dropping from the 20 nip between the chilled rolls 1a and 1b has ceased at the beginning of the casting, the metal solidified at the nip between the chilled rolls 1a and 1b is molded into a strip 8 with a thickness corresponding to the roll gap of the chilled rolls 1a and 1b and is continuously delivered downwardly of the chilled rolls 1a and 1b.

On the other hand, just when the splashing of the molten metal has ceased, the chilled blocks 29a and 29b are moved by the cylinders 24a and 24b to be loosely fitted over the edges 8a and 8b of the strip 8. At the same time, the nitrogen gas is injected as cooling gas through the chilled blocks 29a and 29b. Injection cooling by the nitrogen gas and radiation cooling by the cooling water passing through the chilled blocks 29a and 29b will cool the edges 8a and 8b of the strip 8 positioned near the chilled rolls 1a and 1b.

35 The strip 8 which has been injection- and-radiation-cooled by the chilled blocks 29a and 29b in the chamber 19 with non-oxidizing atmosphere, is guided substantially horizontally by the sledding table 33 to the pinch rolls 18a and 18b and is sent out of the chamber 19 through the pinch rolls 18a and 18b.

When the strip 8 is started to be sent out of the chamber 19, the sledding table 33 is swung to the above-mentioned standby position.

Using the twin roll continuous casting installation shown 45 in FIG. 1, investigation was made on a relationship of perfect solid phase shell thickness near the edge of the strip 8 of distance from the nip between the chilled rolls 1a and 1b in the following respective cases under the manufacturing conditions that strip thickness is 2 mm, manufacturing speed is 60 m/min and atmosphere temperature is 1200° C.:

(1) No cooling is performed on the strip 8.

(2) The strip 8 is injection-cooled by nitrogen gas injected through the cooling gas passages 31a and 31b of the chilled blocks 29a and 29b at a flow rate of 150 m/sec and is radiation-cooled by the cooling water continuously passed through the cooling medium passages 32a and 32b.

(3) The strip 8 is injection-cooled by nitrogen gas injected through the cooling gas passages 31a and 31b of the chilled blocks 29a and 29b at a flow rate of 300 m/sec and is radiation-cooled by the cooling water continuously passed through the cooling medium passages 32a and 32b.

As a result, as shown in FIG. 6, compared with the case 65 1 where no cooling is performed, decrease of perfect solid phase shell thickness of the edge of the strip 8 due to heat recuperation of the unsolidified portion in the strip 8 tends

to be suppressed in the cases 2 and 3 where injection and radiation coolings were carried out near the nip between the chilled rolls 1a and 1b.

In a range investigated, the more the flow rate of the nitrogen gas is, the more the strip 8 is accelerated in 5 solidification.

As described above, in the twin roll continuous casting installation shown in FIGS. 1 to 5, in the chamber 19 with non-oxidizing atmosphere, the edges 8a and 8b of the strip positioned near the chilled rolls 1a and 1b are injection-cooled by the nitrogen gas injected through the cooling gas passages 31a and 31b of the chilled blocks 29a and 29b and are radiation-cooled by the cooling water passed through the cooling medium passages 32a and 32b of the chilled blocks 29a and 29b. Therefore, any decrease of perfect solid phase shell thickness of the strip 8 at its edges 8a and 8b caused by heat recuperation of unsolidified portion can be prevented, and edge bulging and breakout of the strip 8 can be suppressed.

In the twin roll continuous casting installation shown in FIGS. 1 to 5, the chilled blocks 29a and 29b may be moved to the positions where the chilled blocks are not affected by splashing of the molten metal dropping from the nip between the chilled rolls 1a and 1b. As a result, the chilled blocks 29a and 29b can be prevented from being damaged.

It is of course to be understood that the twin roll continuous casting installation of the present invention is not limited to the above embodiment and that various changes and modifications may be made without departing from the spirit and the scope of the invention. For example, in lieu of the nitrogen gas, argon or helium gas may be used as inert gas 30 for attainment of non-oxidizing atmosphere in the chamber as well as for injection cooling of the strip.

#### [Effect of the Invention]

As described above, according to a twin roll continuous casting installation of the invention, the following superb effects can be obtained:

- (1) In accordance with the invention cooling gas is injected toward the edges of the strip positioned near the roll nip of the chilled rolls from the chilled blocks positioned just below the respective chilled rolls. Thus, decrease of perfect solid phase shell thickness of the strip due to heat recuperation of the unsolidified portion can be alleviated and edge bulging and breakout of the strip can be suppressed.
- (2) In twin roll continuous casting installations according to a preferred embodiment of the invention in addition to injection of the cooling gas from the chilled blocks to the strip, the cooling medium is passed through the cooling medium passages of the respective chilled blocks to radiation-cool the edges of the strip positioned near the nip between the chilled rolls so that any decrease of perfect solid phase shell thickness of the strip caused by heat recuperation of the unsolidified portion can be alleviated. Accordingly, edge bulging and breakout of the strip can be further effectively suppressed.
- (3) In twin roll continuous casting installations according to other preferred embodiments of the invention, each of the paired chilled blocks may be moved to a position where the chilled block is not affected by splashing of the molten metal dropping from the nip between the chilled rolls. Thus, damage of the chilled blocks due to splashing of the molten metal at the beginning of the strip casting can be prevented.

What is claimed is:

1. A method for producing a continuously cast thin strip of metal, comprising the steps of:  
casting said thin strip between a pair of chilled casting rolls;

transporting said thin strip through a sealed chamber to a set of pinch rolls;

cooling, at a position just below the chilled casting rolls, the edges of the thin strip, at a cooling rate sufficient to substantially eliminate any decrease of perfect solid phase shell thickness of said thin strip caused by heat recuperation of an unsolidified portion of said strip at the edge thereof;

wherein said cooling of said edges of said strip is effected by cooling means, and said method further includes the steps of ascertaining whether splashing of molten metal below the chilled casting rolls is occurring, and after a cessation of splashing has been ascertained, moving said cooling means from a standby position into a position adjacent the edges of the strip, whereby cooling of said edges is effected.

2. A method as claimed in claim 1, wherein said cooling means comprises a pair of blocks shaped for loose fitting over the edges of the strip, and said moving of said cooling means into a position adjacent the edges of the strip comprises loosely fitting the blocks over the edges of the strip.

3. A method for producing a continuously cast thin strip of metal, comprising the steps of:

casting said thin strip between a pair of chilled casting rolls;

transporting said thin strip through a sealed chamber to a set of pinch rolls;

cooling, at a position just below the chilled casting rolls, the edges of the thin strip, at a cooling rate sufficient to substantially eliminate any decrease of perfect solid phase shell thickness of said thin strip caused by heat recuperation of an unsolidified portion of said strip at the edge thereof;

wherein said cooling of said edges of said strip is effected by cooling means, and said method further includes the further step of continuously passing a cooling fluid through internal passages in said cooling means; and wherein said cooling means includes means for directing a cooling gas onto the edges of the thin strip, and the method further comprises directing a cooling gas through said cooling means onto said edges of said strip.

4. A method as claimed in claim 3, wherein said cooling means comprises a pair of blocks shaped for loose fitting over the edges of the strip.

5. A method for producing a continuously cast thin strip of metal comprising the steps of:

casting said thin strip between a pair of chilled casting rolls;

transporting said thin strips through a sealed chamber to a set of pinch rolls and

cooling, at a position just below the chilled casting rolls, the edges of the thin strip at a cooling rate sufficient to substantially eliminate any decrease of perfect solid phase shell thickness of said thin strip due to heat recuperation of an unsolidified portion at the edge;

wherein said cooling of the edges of the strip is effected by means of a pair of edge cooling blocks shaped for loose fitting over the edges of the block and internally chilled by a flow of cooling water, and said method includes loosely fitting the blocks over the edges of the strip without contact whereby to cool the edges by radiant heat flow into the chilled blocks.

6. A method as claimed in claim 5, and further comprising additionally cooling the strip edges by directing cooling gas through gas flow passages in the blocks onto those edges.